# EUROPEAN PATENT APPLICATION

(11) **EP 0 674 339 A2**
(43) Date of publication of application: **27.09.1995**
(21) Application number: 95200649.2
(22) Date of filing: 17.03.1995
(51) Int. Cl.: H01J 65/04, H01J 61/35, H01J 61/48, H01J 61/44

(54) **Electrodeless low-pressure mercury vapour discharge lamp**

(30) Priority: 25.03.1994 EP 94200806
(71) Applicant: Philips Electronics N.V., 5621 BA Eindhoven (NL)
(72) Inventor: Schlejen, Jakob, NL-5656 AA Eindhoven (NL); Buck, Johannes Jacobus Maria, NL-5656 AA Eindhoven (NL); Roozekrans, Christianus Josephus, NL-5656 AA Eindhoven (NL)
(74) Representative: Evers, Johannes Hubertus Maria

(57) **Abstract**

An electrodeless low-pressure mercury vapor discharge lamp of the invention comprises a discharge vessel (1) that gas-tightly encloses a discharge-space (2) that is provided with a fill of mercury and a noble gas. The discharge vessel (1) has a light-transmitting enveloping part (3A) and further has a sunken part (3B) in which a coil (10) for generating a high-frequency magnetic field is arranged. At least a portion (5B) of a surface (4) of the discharge vessel (1) turned towards the discharge space (2) is provided with a luminescent layer (5A, 5B). At least a portion of the luminescent layer (5B) bears a protective layer (6B) of aluminum oxide particles with a covering weight of 10 to 500 µg/cm². The protective layer provides for a lower mercury consumption and/or a reduction in the change of colour point during lamp life.

## Description

The invention relates to an electrodeless low-pressure mercury vapour discharge lamp with a discharge vessel which encloses a discharge space provided with a filling of mercury and rare gas in a gastight manner, which discharge vessel comprises a light-transmitting enveloping portion and in addition a recessed portion in which a coil for generating a high-frequency magnetic field is enclosed, and which discharge vessel is provided with a luminescent layer at least on a portion of a surface facing towards the discharge space.

Such a lamp is known from EP 0.162.504 B1. The lamp is operated in that the coil is connected to a high-frequency electric supply source. The magnetic field generated by the coil induces an electric discharge in the discharge space. The coil in addition generates a comparatively strong electric field in the discharge space as a result of potential differences across this coil. The electric field strength may be very great especially near the recessed portion of the discharge vessel. In addition, comparatively high temperatures prevail in the wall of the discharge vessel. The temperature of the recessed portion may even assume values above 200° C.

Under these circumstances, luminescent materials present in the luminescent layer may react with particles from the discharge space which collide with these materials. Depending on the application of the lamp, this may give rise to disadvantages.

Usually, several kinds of luminescent materials are present in the luminescent layer, and the luminous efficacies of these materials are affected by the reactions with the particles to different degrees. The result of this is that the colour point of the light generated by the luminescent layer shows a shift during lamp life. This is no disadvantage when a single lamp is used because this process takes place gradually. Even a comparatively great difference with the colour point at the beginning of lamp life is not observable in that case. Clear differences in colour point, however, are observable in applications where known lamps of mutually differing ages are positioned in one and the same space. If one of the lamps is defective, it is necessary to replace not only the defective lamp, but also the other lamps in said space in order to avoid colour point differences under these circumstances, which is expensive. It was found that differences between colour points are observable when at least one of the colour points is present outside the Von Kries transformed MacAdam ellipse of another colour point (see: New Insights in Chromaticity and Tolerance Areas of Fluorescent Lamps, J.J. Opstelten and G. Rinzema, Journal of the IES, Winter 1987, pp. 117-127). This is the case if there is no ellipse half the size of the transformed MacAdam ellipse which comprises all colour points.

It was found to be favourable to operate the lamp of the kind mentioned in the opening paragraph by means of a pulsatory supply. The lumen output of the lamp may be adjusted between, for example, 10% and 100% of its rated lumen output in this mode of operation in that the ratio of the pulse duration to the time interval between the pulses is varied. In this mode of operation, however, comparatively high voltages are required for re-igniting the lamp at the start of each pulse. Electric fields will then occur, especially near the recessed portion, which are even stronger than those during nominal operation. It was found that mercury is bound to material in the luminescent layer under these circumstances, which mercury is no longer available for lamp operation. A comparatively large quantity of mercury is necessary if a sufficiently long lamp life is to be guaranteed in spite of this. This is bad for the environment in the case of inexpert disposal at the end of lamp life.

The invention has for its object to provide a measure in an electrodeless low-pressure mercury vapour discharge lamp of the kind described in the opening paragraph which counteracts the interaction between the luminescent layer and particles from the discharge space.

The electrodeless low-pressure mercury vapour discharge lamp according to the invention is for this purpose characterized in that at least a portion of the luminescent layer bears a protective layer of aluminium oxide particles with a coating weight of 10 to 500 µg/cm². It was surprisingly found that this measure counteracts the interaction between the luminescent layer and particles from the discharge space in spite of the comparatively strong electric fields and the comparatively high temperatures prevalent in the lamp.

It is noted that US 4,639,637 discloses a low-pressure mercury vapour discharge lamp with a tubular discharge vessel which is provided with a luminescent layer coated with an aluminium oxide layer at a surface facing towards the discharge space. In contrast to the lamp according to the invention, however, the lamp is ignited and the discharge is maintained by a pair of electrodes arranged in the discharge vessel. The electric fields occurring near the luminescent layer are weak in such lamps. The temperatures prevalent in the discharge vessel wall are comparatively low.

A first attractive embodiment of the lamp according to the invention is characterized in that the surface of the recessed portion facing towards the discharge space is provided with a luminescent layer which bears a protective layer having a coating weight of 100 to 500 µg/cm². This embodiment of the lamp according to the invention has the advantage that only little mercury is bound by the luminescent layer also during operation by means of a pulsatory supply. A luminescent layer on the enveloping portion of the discharge vessel is, for example, absent. The lamp may then be used as a UV radiator.

A second attractive embodiment is characterized in that the surface of the enveloping portion facing towards the discharge space is provided with a luminescent layer bearing a protective layer having a coating weight of 10 to 50 µg/cm². Lamps according to this embodiment of the invention have the advantage that the colour point shift is so small that no difference is perceivable between the colour points of lamps of the same embodiment but differing in age. The recessed portion may be provided, for example, with a reflecting layer. In a modification, the recessed portion is also provided with a luminescent layer. It was found in this modification of the second embodiment that the colour point shift is also very small without a protective layer on the luminescent layer of the recessed portion. It is favourable, however, if the luminescent layer on the recessed portion bears a protective layer corresponding to that of the first embodiment in this modification. The lamp is then also suitable for pulsatory operation.

The protective layer may be readily provided in the form of a suspension of aluminium oxide powder, after which the layer is sintered, *i.e.* is heated for some time in order to drive out auxiliary substances such as binders from the layer. The suspension is applied to the surface, for example, by spraying. For providing the protective layer on the recessed portion, it may suffice to immerse the recessed portion in the suspension. Alternatively, the layer may be provided, for example, through electrostatic coating.

It is found in practice that lamp characteristics of electrodeless lamps, such as the lumen output or the change therein during lamp life, depend on the production location of the lamp.

It was surprisingly found with the lamp according to the invention that the change in lumen output depends much less on the production location than with the lamp not according to the invention. The measure according to the invention thus improves the reproducibility of said lamp characteristic in the case of manufacture in different locations.

Embodiments of the electrodeless low-pressure mercury vapour discharge lamp according to the invention are explained in more detail with reference to the drawings, in which:
Figs. 1 and 2 show a first and a second embodiment of the lamp, respectively, partly in side elevation and partly in longitudinal sectional view. A supply device is also shown diagrammatically.
Figs. 3 and 4 show the colour point shift of lamps according to the second embodiment and of lamps not according to this embodiment, respectively.

The embodiment of the electrodeless low-pressure mercury vapour discharge lamp according to the invention shown in Fig. 1 is provided with a pearshaped, gastight discharge vessel 1 which encloses a discharge space 2. The discharge vessel 1 has a light-transmitting enveloping portion 3A and a tubular, recessed portion 3B. The discharge vessel 1 further has a flanged portion 3C which connects the recessed portion 3B to the enveloping portion 3A. The discharge space 2 is provided with a filling of mercury and a rare gas, here argon. A coil 10 for generating a high-frequency magnetic field is accommodated in the recessed portion 3B. The coil 10 has a length of 25 mm and is provided with a first and a second winding 11, 12, each of 15 turns around a core 13 of soft-magnetic material. In an alternative embodiment, the coil may have, for example, an air core, or a core of ceramic material. The first winding 11 is connected to a high-frequency supply source 20 by means of current supply conductors 14, 15 in order to operate the lamp. The supply source 20 here has a frequency of 2.65 MHz. The second winding 12 has an end which is connected to current supply conductor 15 and also has a further, free end. The supply source 20 is connected to poles P and N of the mains and is earthed at pole M. The recessed portion 3B of the discharge vessel 1 is provided with a luminescent layer 5B at a surface 4 facing towards the discharge space 2, this layer comprising red-luminescing yttrium oxide activated by trivalent europium (YOX) and green-luminescing cerium-magnesium aluminate activated by trivalent terbium (CAT). The luminescent layer 5B has a coating weight of 8 mg/cm². A surface 4 of the enveloping portion 3A facing towards the discharge space 2 is provided with a luminescent layer 5A which comprises blue-luminescing barium-magnesium aluminate activated by bivalent europium (BAM) in addition to the luminescent materials YOX and CAT. This luminescent layer 5A has a coating weight of 3.5 mg/cm².

The luminescent layer 5b on the surface 4 of the recessed portion 3B facing towards the discharge space 2 bears a protective layer 6B of aluminium oxide particles. The protective layer 6B was obtained in this case in that the recessed portion 3B was immersed in a suspension of Alon-C of the Degussa company, after which the layer remaining on the recessed portion 3B was dried and then sintered. The coating weight depends on the concentration of the aluminium oxide powder present in the suspension. Aluminium oxide powder of the Alon-C type comprises aluminium oxide particles with a size of approximately 0.01 to 0.04 µm, and has a specific area of approximately 100 m²/g.

Lamps corresponding to the embodiment shown in Fig. 1 and having a coating weight of 170 µg/cm², of 250 µg/cm², and of 300 µgcm² were manufactured, two of each Kind. The coating weights of the lamps accordingly lay between the limits of 100 and 500 µg/cm². Two reference lamps were also manufactured in which a protective layer of aluminium oxide particles on the luminescent layer of the recessed portion was absent. The six lamps according to the invention and the two reference lamps were subjected to an endurance test of approximately 170 hours in order to assess the influence of strong electric fields of the kind which may arise during re-ignition. Each lamp was provided with a coil whose windings were interrupted for this purpose. The windings jointly extend over a length of 30.5 mm around the coil core. The interruption in the coil creates two coil parts each of 7.5 turns, approximately 5 mm spaced apart. A voltage of 700 V was applied to this coil during the endurance test. Since the coil is interrupted, it does not generate a magnetic field, so that no arc discharge is generated in the discharge vessel. The lamp accordingly remains permanently in a condition corresponding to that during re-ignition in reduced operation during the endurance test. In reduced operation of the lamp, the comparatively high re-ignition voltages occur during a fraction of each cycle only. This is because, on the one hand, a voltage is applied to the coil during a portion of each cycle only in this mode of operation, and on the other hand because the voltage across the coil drops quickly after lamp re-ignition. It is assumed that the above endurance test of 170 hours is comparable to approximately 5000 hours of pulsatory operation with a lamp power which is reduced to 15%.

A strong blackening of the luminescent layer between the coil parts was observed in the reference lamps after this endurance test. In the lamps according to the invention having a coating weight of 170 and 250 µg/cm², the luminescent layer was much less strongly discolored. A discoloration was even substantially absent in the lamps according to the invention having a coating weight of 300 µg/cm².

An electrodeless lamp was manufactured for comparison whose recessed portion was provided with a luminescent layer coated with a silicon oxide layer and one whose luminescent layer on the recessed portion was coated with an yttrium oxide layer. The lamps were also subjected to an endurance test. After no more than 16 hours of operation at a voltage of 600 V, the lamp with the yttrium oxide layer exhibited a pale brown band between the coil parts. The section of the recessed portion lying between the coil parts in the lamp having the silicon oxide layer remained unchanged in colour. The recessed portion, however, did show a grey discoloration on either side thereof.

It was also investigated, after the endurance test had been completed, to what extent mercury was bound to the luminescent material in the lamps according to the invention and in the reference lamps. For that purpose, the section of the recessed portion situated between the coil parts was subjected to a wet chemical analysis.

The average quantity of mercury bound to the wall in the reference lamps (REF) and the respective average quantities in the lamps having a coating weight of 170, 250 and 300 µg/cm² are listed in the following Table.

| coating weight (µg/cm²) | m_{Hg} (µg) |
|---|---|
| REF | 62 |
| 170 | 33 |
| 250 | 30 |
| 300 | 18 |

It is evident from the Table that the quantity of bound mercury in the lamps according to the invention with a protective layer having a coating weight of 170 and 250 µg/cm² is approximately half that of the reference lamps. The quantity of bound mercury is even about one third in the lamp according to the invention whose protective layer has a coating weight of 300 µg/cm².

The drift in the lumen output between 1 and 100 hours of operation was measured for 10 lamps according to the invention whose luminescent layers on the recessed portions were coated with a protective layer of aluminium oxide particles, and for 10 lamps not according to the invention. The lamps not according to the invention correspond to those according to the invention except for the absence of a protective layer. Five of the lamps according to the invention were manufactured in a first production location (A), and five in a second production location (B). Similarly, five of the lamps not according to the invention were manufactured in the first production location (A) and five in the second production location (B).

The drift in the lumen output in the period from 1 to 100 hours of operation is shown in the following Table.

| | Lamp not according to the invention | Lamp according to the invention |
|---|---|---|
| A | 98.2 % | 98.3 % |
| B | 93.7% | 95.7 % |
| difference | 4.5 % | 2.6 % |

Manufacture in different production locations leads to a difference in the lumen output drift of 4.5% in the lamps not according to the invention. This difference is no more than 2.6% in the lamps according to the invention.

In Fig. 2, parts corresponding to those of Fig. 1 have reference numerals which are 100 higher. In the embodiment of the electrodeless low-pressure mercury vapour discharge lamp according to the invention shown here, the surface 104 of the enveloping portion 103A facing the discharge space 102 is provided with a luminescent layer 105A which bears a protective layer 106A with a coating weight of 28 µg/cm². The coating weight accordingly lies within the limits of 10 and 50 µg/cm².

In the embodiment shown, the flanged portion 103C has neither a luminescent nor a protective layer. In a modification, this portion 103C also has a luminescent layer, possibly be provided with a protective layer.

Six lamps were manufactured corresponding to the embodiment of the invention described with reference to Fig. 2.
In addition, five reference lamps were manufactured without a protective layer of aluminium oxide particles on the luminescent layer of the enveloping portion.

The above 11 lamps were subjected to an endurance test. The lamps were switched off for half an hour after 2.5 hours of operation each time during this. The x- and y-coordinates of the colour point were measured for the said lamps both at the start and after 2000 hours of operation. Fig. 3 shows the colour points at the beginning (open dots) and after completion of the endurance test (closed dots) for the six lamps according to the invention. Fig. 4 shows the colour points of the five lamps which do not have a protective layer of aluminium oxide particles on the enveloping portion. In these Figures, the colour points at the beginning of lamp life are indicated with open dots and those at the end of lamp life with closed dots. Only four colour points are visible in Fig. 4 because two colour points had equal coordinates both at the beginning and at the end of the endurance test.

It is evident from Fig. 3 that the colour points of the lamps measured at the start and after completion of the endurance test lie jointly within an ellipse having half the size of a Von Kries transformed MacAdam ellipse. The average deviation of the colour coordinates at the end of the endurance test compared with those at the beginning is 0.001 and 0.003, respectively.

Fig. 4 shows that the colour points of lamps not having a protective layer on the enveloping portion differ considerably after completion of the endurance test from those at the beginning of the endurance test. The average deviation of the x- and y-coordinates is 0.017 and 0.010, respectively.

It is clear from the above that lamps corresponding to the embodiment of the invention described with reference to Fig. 2 show only a very small drift in their colour point compared with lamps not corresponding to said embodiment. The average initial value of the colour point (x = 375, y = 383) differs slightly from the average initial value of the colour point (x = 381, y = 379) of the lamp not corresponding to said embodiment. This difference in the initial value of the colour point may easily be eliminated by means of a minor change in the composition of the luminescent layer.

## Claims

1. An electrodeless low-pressure mercury vapour discharge lamp with a discharge vessel (1) which encloses a discharge space (2) provided with a filling of mercury and rare gas in a gastight manner, which discharge vessel (1) comprises a light-transmitting enveloping portion (3A) and in addition a recessed portion (3B) in which a coil (10) for generating a high-frequency magnetic field is enclosed, and which discharge vessel (1) is provided with a luminescent layer (5A, 5B) at least on a portion of a surface (4) facing towards the discharge space (2), characterized in that at least a portion of the luminescent layer (5B) bears a protective layer (6B) of aluminium oxide particles with a coating weight of 10 to 500 µg/cm².

2. An electrodeless low-pressure mercury vapour discharge lamp as claimed in Claim 1, characterized in that the surface (4) of the recessed portion (3B) facing towards the discharge space (2) is provided with a luminescent layer (5B) which bears a protective layer (6B) having a coating weight of 100 to 500 µg/cm².

3. An electrodeless low-pressure vapour discharge lamp as claimed in Claim 1 or 2, characterized in that the surface (104) of the enveloping portion (103A) facing towards the discharge space (102) is provided with a luminescent layer (105A) bearing a protective layer (106A) having a coating weight of 10 to 50 µg/cm².
